

Sept. 24, 1929.

C. A. PARSONS ET AL

1,729,009

MANUFACTURE OF METAL STRIP SUITABLE FOR TURBINE BLADES

Filed Jan. 21, 1928



Fig. 1.



Fig. 3.



Fig. 2.

Inventors

Charles A. Parsons  
Edward G. Brownlow

*By Spear, Middleton, Dacoror & Hays*

## UNITED STATES PATENT OFFICE

CHARLES ALGERNON PARSONS AND EDWARD GARRETT BROWNLOW, OF NEWCASTLE-ON-TYNE, ENGLAND; SAID BROWNLOW ASSIGNEE TO SAID PARSONS

## MANUFACTURE OF METAL STRIP SUITABLE FOR TURBINE BLADES

Application filed January 21, 1928, Serial No. 248,426, and in Great Britain February 7, 1927.

The invention relates to the manufacture of metal strip by an extension process such as rolling and is specially applicable to the rolling of metal strip for turbine blades.

5 In the particular case of reaction turbine blades formed integral with their roots by a rolling process, the blank or billet has a root-forming portion approximating to the final form and a tail portion to be extended and shaped by rolling to form the strip-like projection constituting the blade proper. If as is usual the blade-forming portion of the billet is formed for convenience of rectangular or other simple section, it is found that the blade 10 curves to one side during the rolling process owing to the greater extension of that part of the billet which forms the thinner edge.

When strip is rolled in long lengths no particular difficulty is found in providing 20 guides to keep it straight, but in short lengths and particularly as above where each blade is integral with its root such guiding is practically out of the question.

The main object of the present invention is 25 to overcome such difficulties.

The invention consists in the process of manufacturing metal bar as hereinafter described and particularly set forth in the claims.

30 Referring to the accompanying drawings, which illustrate diagrammatically one form of the invention:—

Figure 1 shows in full lines a turbine-blade blank or billet suitable for a cylindrical rotor and having a curved blade-forming portion, the finished blade being indicated by dotted lines,

Figure 2 being a section on the line 2—2 of Figure 1; while

40 Figure 3 shows a modified form of blank suitable for a conical rotor.

In carrying the invention into effect according to the form shown as applied by way of example to the production of reaction turbine blading, the blank or billet (see Figures 1 and 2) has a rectangular root-forming base, *a*, of uniform thickness and a blade-forming tail, *b*, of rectangular cross section projecting from a side of the base and of the same 50 thickness as the base. The blade-forming

portion, *b*, of the blank instead of coinciding in direction with the finished blade is curved as a whole (see the full lines in Figure 1) to that side on which the thinner edge, *b'*, of the finished blade will be formed.

If the initial curvature of the blank is properly chosen the extra extension of that side of the blade-forming portion which corresponds to the thinner edge, *b'*, of the finished blade will cause the blank to become less 55 curved during each rolling operation and finally to become straight, as shown by the dotted lines in Figure 1.

The blank as described above with a rectangular base is suitable for cylindrical rotors or stators but the root-forming portion may be modified, for example as shown at *a'*, in Figure 3, to render it suitable for conical rotors and stators or other constructions.

We wish it to be understood that the invention may be applied to other purposes than turbine blades while the details of its performance described above may be varied 70 to suit particular cases.

It will be understood that the blank is 75 differentially extended longitudinally owing to the fact that the rolls have a gap between them of the non-symmetrical cross section required, and that the blank is of rectangular or other simple cross section.

By differential extension is meant the longitudinal extension of one side of the symmetrical blank more than the other side thereof. That is, the curved blank of rectangular cross-section, when subjected to 85 gap-rolling, will straighten out due to the extension of the concave side of the curved blank more than the convex side, the concave side being rolled thinner than the convex side.

This variation in longitudinal extension from one side of the blank to the other being gradual is termed differential extension as defining the variation in extension by increments from one side to the other.

Having now described our invention, what we claim as new and desire to secure by Letters Patent is:—

1. A process of manufacturing metal bar 100 of non-symmetrical cross section, which con-

sists in preparing a curved billet and reducing the curvature of said billet by differentially extending said billet longitudinally to give the non-symmetrical cross section required, the concave side of said curved billet being extended more than the convex side.

2. A process as claimed in claim 1, in which the cross section of the curved billet is initially uniform.

10 3. A process of manufacturing turbine blading having a non-symmetrical cross section with a thicker and a thinner edge, which consists in preparing a billet curved towards that side of the billet which will 15 correspond to said thinner edge of the finished blade and reducing the curvature of said billet by differentially extending said billet longitudinally to give the non-symmetrical cross section required, the concave 20 side of said curved billet being extended more than the convex side.

4. A process of manufacturing turbine blading having a non-symmetrical cross section with a thicker and a thinner edge and 25 an integral base, which consists in preparing a billet having a base-forming portion and a blade-forming portion integral with said base-forming portion and curved towards that side of the billet which will corre- 30 spond to said thinner edge of the finished blade and reducing the curvature of said blade-forming portion of the billet by differentially extending said blade-forming portion only of said billet longitudinally to 35 give the non-symmetrical cross section required, the concave side of said curved billet being extended more than the convex side.

In testimony whereof we have signed our names to this specification.

40 CHARLES ALGERNON PARSONS.  
EDWARD GARRETT BROWNLOW.

45

50

55

60

65